



US010722935B2

(12) **United States Patent**  
**Furusako et al.**

(10) **Patent No.:** **US 10,722,935 B2**  
(45) **Date of Patent:** **\*Jul. 28, 2020**

(54) **MECHANICAL JOINING APPARATUS AND MECHANICAL JOINING METHOD**

(71) Applicant: **NIPPON STEEL CORPORATION**,  
Tokyo (JP)

(72) Inventors: **Seiji Furusako**, Tokyo (JP); **Tohru Okada**, Tokyo (JP); **Yasunobu Miyazaki**, Tokyo (JP); **Fuminori Watanabe**, Tokyo (JP); **Yoshiaki Nakazawa**, Tokyo (JP)

(73) Assignee: **NIPPON STEEL CORPORATION**,  
Tokyo (JP)

(\*) Notice: Subject to any disclaimer, the term of this patent is extended or adjusted under 35 U.S.C. 154(b) by 91 days.

This patent is subject to a terminal disclaimer.

(21) Appl. No.: **15/740,786**

(22) PCT Filed: **Jul. 1, 2016**

(86) PCT No.: **PCT/JP2016/069718**

§ 371 (c)(1),  
(2) Date: **Dec. 28, 2017**

(87) PCT Pub. No.: **WO2017/002975**

PCT Pub. Date: **Jan. 5, 2017**

(65) **Prior Publication Data**

US 2018/0185902 A1 Jul. 5, 2018

(30) **Foreign Application Priority Data**

Jul. 1, 2015 (JP) ..... 2015-133106

(51) **Int. Cl.**

**B21J 15/08** (2006.01)  
**B21J 15/02** (2006.01)

(Continued)

(52) **U.S. Cl.**

CPC ..... **B21J 15/025** (2013.01); **B21J 15/08** (2013.01); **B21J 15/28** (2013.01); **B21J 15/30** (2013.01); **B21J 15/36** (2013.01)

(58) **Field of Classification Search**

CPC combination set(s) only.  
See application file for complete search history.

(56)

**References Cited**

**U.S. PATENT DOCUMENTS**

6,108,890 A \* 8/2000 Opper ..... B21J 15/025  
29/413  
6,417,490 B1 7/2002 Liebrecht et al.  
(Continued)

**FOREIGN PATENT DOCUMENTS**

CN 101716644 A 6/2010  
CN 101920302 A 12/2010  
(Continued)

**OTHER PUBLICATIONS**

Extended European Search Report, dated Jan. 25, 2019, for European Application No. 16818083.4.

(Continued)

*Primary Examiner* — Jun S Yoo

(74) *Attorney, Agent, or Firm* — Birch, Stewart, Kolasch & Birch, LLP

(57) **ABSTRACT**

Provided is a mechanical joining apparatus enabling stable riveting when joining metal sheets even when the sheets are large in deformation resistance, the apparatus comprising a punch and die, blank holder and power device, wherein the punch and die are arranged facing each other, the holder is configured by an electrode material able to push against and electrically heat the sheets by one end of the holder, the punch is comprised of a material able to drive in a rivet, the die is comprised of an electrode material able to support and electrically heat the sheets, and the power device is configured to start supply of current through the holder and die so

(Continued)



as to raise the temperature of the sheets at the same time as the start of driving in of the rivet and to continue to supply current until the end of driving in of the rivet.

**7 Claims, 3 Drawing Sheets**

(51) **Int. Cl.**  
*B21J 15/28* (2006.01)  
*B21J 15/30* (2006.01)  
*B21J 15/36* (2006.01)

(56) **References Cited**

U.S. PATENT DOCUMENTS

|                  |        |                                          |
|------------------|--------|------------------------------------------|
| 6,694,597 B2     | 2/2004 | Wang et al.                              |
| 2003/0167621 A1* | 9/2003 | Wang ..... B21J 15/025<br>29/525.06      |
| 2004/0148760 A1* | 8/2004 | Wang ..... B21J 15/025<br>29/525.06      |
| 2005/0161965 A1* | 7/2005 | Eberlein ..... B21J 15/025<br>296/29     |
| 2010/0018027 A1* | 1/2010 | Stevenson ..... B21J 15/025<br>29/525.06 |

|                  |         |                                        |
|------------------|---------|----------------------------------------|
| 2010/0083481 A1* | 4/2010  | Luo ..... B21J 15/025<br>29/432        |
| 2014/0290064 A1* | 10/2014 | Smeijers ..... B21J 15/025<br>29/897.2 |
| 2016/0262214 A1  | 9/2016  | Kondo et al.                           |

FOREIGN PATENT DOCUMENTS

|    |                   |         |
|----|-------------------|---------|
| CN | 103600017 A       | 2/2014  |
| DE | 10060390 A1       | 6/2002  |
| EP | 2514537 A1        | 10/2012 |
| JP | 2000-202563 A     | 7/2000  |
| JP | 2004-516140 A     | 6/2004  |
| JP | 2006-7266 A       | 1/2006  |
| JP | 2007-521964 A     | 8/2007  |
| JP | 2007-254775 A     | 10/2007 |
| WO | WO 2014/196268 A1 | 12/2014 |
| WO | WO 2015/075964 A1 | 5/2015  |

OTHER PUBLICATIONS

Abe, "Joining of Sheets by Self Piercing Rivet and Mechanical Clinch," Ferrum, vol. 16, No. 9, 2011, pp. 32-38.  
 International Search Report for International Application No. PCT/JP2016/069718, dated Oct. 4, 2016, with English translation.

\* cited by examiner

FIG. 1



FIG. 2



FIG. 3



## 1

MECHANICAL JOINING APPARATUS AND  
MECHANICAL JOINING METHOD

## TECHNICAL FIELD

The present disclosure relates to a mechanical joining apparatus able to be used when joining a plurality of metal sheets and the metal sheets are large in deformation resistance, more particularly relates to a mechanical joining apparatus able to be used when the plurality of metal sheets includes one or more high strength steel sheets with a tensile strength of 780 MPa or more or when even if the metal sheets are small in tensile strength, the processing speed is large.

## BACKGROUND ART

In recent years, in the automotive field, to lower fuel consumption and cut the amount of emission of CO<sub>2</sub>, it has been demanded to make the car bodies lighter in weight while improving impact safety by making the car body members high in strength. To meet these demands, it is effective to use high strength steel sheet for the car bodies and parts. For this reason, demand for high strength steel sheet has been rising. To use high strength steel sheet for car bodies or parts etc., the high strength steel sheet has to be joined with other metal sheets, but there are the following such problems in joining them.

In the past, car bodies have been assembled and parts attached etc. mainly by spot welding. Spot welding has been employed even when joining a plurality of metal sheets including high strength steel sheets. In a joint formed by superposing a plurality of metal sheets and spot welding them in this way, the tensile strength is an important characteristic. As the tensile strength, there are a tensile shear strength (TSS) measured by applying a tensile load in the shear direction and a cross tensile strength (CTS) measured by applying a tensile load in the peeling direction.

A spot welded joint formed from a plurality of steel sheets having a 270 to 600 MPa tensile strength increases in CTS along with an increase in strength of the steel sheets. Therefore, in a spot welded joint formed by steel sheets having a 270 to 600 MPa tensile strength, problems relating to joint strength seldom occur. However, in a spot welded joint formed by a plurality of metal sheets including one or more steel sheets having a 780 MPa or more tensile strength, even if the steel sheets increase in tensile strength, the CTS does not increase or else decreases. This is because due to the drop in deformation ability, more stress concentrates at the weld zones, due to inclusion of large amounts of alloy elements, the weld zones are hardened, and due to segregation by solidification, the weld zones fall in toughness.

For this reason, in joining a plurality of metal sheets including one or more steel sheets having a 780 MPa or more tensile strength, art for improving the CTS has been sought. As one of the arts for solving this problem, there is the art of mechanical joining members without causing the matrix material to melt. Specifically, there is the art of stacking members to be joined such as a plurality of metal sheets, holding down the outer circumference of the punch by a blank holder preventing the metal sheets from springing up while driving in a rivet by the punch, and thereby mechanically joining the plurality of metal sheets with each other by the rivet.

However, in this art, there were the problem that since a rivet is driven in, the die side steel sheet deforms by an extremely great amount and, due to insufficient ductility or

## 2

localization of deformation, the die side steel sheet fractures, the problem that when a tensile stress is applied in the shear direction and peel direction, the rivet will pull out and break and sufficient values of tensile strength in the shear direction and peel direction cannot be obtained, and the problem that there is almost no difference from the same rivet driving type of high strength steel sheet joints and mild steel sheet joints when comparing the fatigue strengths of the two.

As art for solving such problems, PLT 1 discloses the art of joining stacked high strength steel sheets with tensile strengths of 430 to 1000 MPa by driving a rivet through them and deforming the emerging front end of the rivet to thereby mechanically join the sheets and obtain a high strength steel sheet excellent in tensile properties and fatigue properties. The art disclosed in PLT 1 covers high strength steel sheet with a tensile strength of up to 619 MPa in its study and is effective as art when joining a plurality of steel sheets. However, in PLT 1, application of the above art to a plurality of steel sheets including high strength steel sheets with a tensile strength of 780 MPa or more was not studied.

Further, NPLT 1 describes that when joining high strength steel sheet and aluminum alloy sheet by driving in a rivet to mechanically join them, joining them without defect is possible up to a plurality of metal sheets including high strength steel sheet with a tensile strength of 590 MPa or so, but with a plurality of metal sheets including high strength steel sheet with a tensile strength of 980 MPa, the rivet cannot pierce through the high strength steel sheet.

In this way, in the art of driving a rivet into metal sheets to mechanically join them, usually a hole is not drilled into the members to be joined before joining them but the rivet itself is used to pierce through the members to be joined, so it was considered difficult to drive a rivet through a plurality of metal sheets including one or more steel sheets with a large deformation resistance, for example, steel sheets with a 780 MPa or more tensile strength, to mechanically join them.

As opposed to this, PLT 2 discloses a mechanical joining method joining thin-gauge sheets having high strength or work hardened to a high degree using a rivet wherein at the start of the joining process or right before it, a blank holder and die or components arranged next to the blank holder and die or components arranged in front of them are used to heat the thin gauge sheets restricted in location and time by electrical resistance heating.

In this way, PLT 2 describes art able to be applied to steel sheet having a high strength or work hardened to a high extent. It can be considered art effective to a certain extent even for a plurality of metal sheets including one or more high strength steel sheets with a tensile strength of 780 MPa or more. However, when using the art disclosed in PLT 2 to actually join together by a rivet a plurality of metal sheets including one or more high strength steel sheets with a tensile strength of 780 MPa or more, sometimes riveting is not possible. There was room for further improvement. Further, even with a metal sheet with a tensile strength of less than 780 MPa, if the processing speed when driving in the rivet becomes higher, the metal sheet becomes larger in deformation resistance and therefore similarly there was room for improvement.

## CITATION LIST

## Patent Literature

NPLT 1: Ferrum, Vol. 16 (2011), No. 9, p. 32-38

## SUMMARY OF THE INVENTION

## Problems to be Solved by the Invention

The present disclosure, in view of the current state of the prior art described above, has as its object the provision of a mechanical joining apparatus and mechanical joining method enabling stable riveting when joining a plurality of metal sheets even when the metal sheets are large in deformation resistance.

## Means for Solving the Problems

Therefore, the inventors studied intensively methods for solving the above problems. In the art disclosed in PLT 2, the heating temperature of the steel sheets was made 35 to 250° C. and the steel sheets finished being heated before driving in the rivet. Therefore, the inventors came up with the idea of driving in the rivet while heating the plurality of metal sheets at the time of riveting when the metal sheets are large in deformation resistance.

As a result, they discovered that there was no fracture of the metal sheets, breakage of rivets, failure of rivet piercing, etc. Further, they came up with the idea of supplying a current between the blank holder and die while driving the rivet into the plurality of metal sheets so as to raise the temperature of the plurality of metal sheets.

The mechanical joining apparatus and mechanical joining method of the present disclosure were made based on the above discovery and have as their gists the following:

(1) A mechanical joining apparatus using a punch to drive a rivet into a plurality of metal sheets,

the mechanical joining apparatus comprising a punch and die, a blank holder, and a first power device, wherein

the punch and die are arranged facing each other so as to enable the punch and die to sandwich a superposed plurality of metal sheets between the punch and die,

the blank holder is a tubular member inside of which the punch can be inserted and is configured by an electrode material able to push against the plurality of metal sheets and able to electrically heat the plurality of metal sheets by one end of the blank holder being made to contact a punch side metal sheet of the plurality of metal sheets,

the punch is comprised of a material able to drive in a rivet,

the die is comprised of an electrode material able to support the plurality of metal sheets and able to electrically heat the plurality of metal sheets, and

the first power device is configured to start supply of current through the blank holder and the die so as to raise the temperature of the plurality of metal sheets at the same time as the start of the driving in of the rivet by the punch and to continue to supply current through the blank holder and the die until the end of the driving in of the rivet.

(2) The mechanical joining apparatus according to (1), wherein the mechanical joining apparatus further comprises a cooling device, and the cooling device is connected to the punch and is configured to cool the rivet in a period from the start of the driving in of the rivet to the end of the driving in of the rivet.

(3) The mechanical joining apparatus according to (1) or (2), wherein

the punch is configured by an electrode material able to drive in the rivet and able to electrically heat the rivet,

5 a second power device is configured to supply current through the punch and the die so as to supply current through the rivet and heat treat the rivet after the punch is used to drive in the rivet, and

the mechanical joining apparatus further comprises a cooling device, the cooling device being configured to cool the rivet after heat treatment of the rivet.

(4) The mechanical joining apparatus according to any one of (1) to (3), wherein in the die, at least a part facing the rivet across the plurality of metal sheets is made of tool steel and a part at the outer circumference of the tool steel is made of copper or copper alloy.

(5) A mechanical joining method using a punch to drive a rivet into a plurality of metal sheets, the mechanical joining method comprising

preparing a plurality of metal sheets,

placing the plurality of metal sheets stacked between a punch and die arranged facing each other,

25 pushing one end of a blank holder comprised of a tubular member inside of which the punch can be inserted against a punch side metal sheet of the plurality of metal sheets,

using the punch to drive a rivet into the plurality of metal sheets held by the blank holder, and

30 starting to electrically heat the plurality of metal sheets through the blank holder and the die so as to raise the temperature of the plurality of metal sheets at the same time as the start of the driving in of the rivet and continuing to electrically heat the plurality of metal sheets until the end of the driving in of the rivet.

(6) The mechanical joining method according to (5), further comprising cooling the rivet through the punch in a period from the start of the driving in of the rivet until the end of the driving in of the rivet.

(7) The mechanical joining method according to (5) or (6), further comprising, after driving in the rivet, electrically heating the rivet through the punch and the die to heat treat the rivet, then cooling the rivet.

(8) The mechanical joining method according to any one of (5) to (7), wherein in the die, at least a part facing the rivet across the plurality of metal sheets is made of tool steel and a part at the outer circumferences of the tool steel is made of copper or copper alloy.

## Effect of the Invention

According to the mechanical joining apparatus and mechanical joining method of the present disclosure, it is possible to obtain a joint without fracture of the metal sheets, breakage of the rivets, or failure of rivet piercing even when the metal sheets are large in deformation resistance.

## BRIEF DESCRIPTION OF THE DRAWINGS

FIGS. 1A and 1B are cross-sectional schematic views showing modes of mechanical joining.

FIG. 1A is a cross-sectional schematic view showing the state when starting to electrically heat a set of sheets simultaneously with the start of an operation to drive in a rivet.

## 5

FIG. 1B is a cross-sectional schematic view showing the state after driving in the rivet.

FIGS. 2A and 2B are cross-sectional schematic views showing modes of mechanical joining.

FIG. 2A is a cross-sectional schematic view showing the state when starting to electrically heat a set of sheets simultaneously with the start of an operation to drive in a rivet.

FIG. 2B is a cross-sectional schematic view showing the state when electrically heating a rivet after driving in the rivet.

FIGS. 3A and 3B are cross-sectional schematic views showing modes of mechanical joining in the case of using tool steel for part of the die.

FIG. 3A is a cross-sectional schematic view showing the state when electrically heating a set of sheets simultaneously with the start of an operation to drive in a rivet when using tool steel for part of the die.

FIG. 3B is a cross-sectional schematic view showing the state when electrically heating a rivet after driving in the rivet when using tool steel for part of the die.

## DESCRIPTION OF EMBODIMENTS

The inventors used the art disclosed in PLT 2 and ran a current between a blank holder and a die set at an opposite side to a punch, arranged so as to sandwich a plurality of metal sheets (below, also referred to as a "set of sheets") including high strength steel sheet with a tensile strength of 780 MPa or more (below, also referred to as "high strength steel sheet"), to electrically heat the set of sheets and drove in a rivet, but sometimes riveting was not possible. Further, when using metal sheets with a tensile strength of only less than 780 MPa, if increasing the working speed when driving in a rivet, the metal sheets became greater in deformation resistance and sometimes riveting was not possible.

The inventors took note of the fact that in the art disclosed in PLT 2, the heating temperature of the steel sheet was made 35 to 250° C. and the heating of the steel sheet was ended before driving in the rivet and came up with the idea of, when riveting, heating the set of sheets while driving in the rivet.

The inventors heated sets of sheets of various combinations of metal sheets while driving in rivets and investigated the relationship with rivet breakage etc. As a result, they discovered that by raising the temperature of the set of sheets at the same time as the start of an operation to drive a rivet into the set of sheets, stable riveting is possible. Furthermore, they came up with the idea of raising the temperature of the set of sheets by supplying a current between the blank holder and die and thereby discovered the mechanical joining apparatus of the present disclosure (below, also referred to as the "joining apparatus").

The present disclosure covers a mechanical joining apparatus using a punch to drive a rivet into a plurality of metal sheets, the mechanical joining apparatus comprising

a punch and die,

a blank holder, and

a first power device, wherein

the punch and die are arranged facing each other so as to enable the punch and die to sandwich a superposed plurality of metal sheets between the punch and die,

the blank holder is a tubular member inside of which the punch can be inserted and is configured by an electrode material able to push against the plurality of metal sheets and able to electrically heat the plurality of metal sheets by one

## 6

end of the blank holder being made to contact a punch side metal sheet of the plurality of metal sheets,

the punch is comprised of a material able to drive in a rivet,

the die is comprised of an electrode material able to support the plurality of metal sheets and able to electrically heat the plurality of metal sheets, and

the first power device is configured to start supply of current through the blank holder and the die so as to raise the temperature of the plurality of metal sheets at the same time as the start of the driving in of the rivet by the punch and to continue to supply current through the blank holder and the die until the end of the driving in of the rivet.

Below, while referring to the figures, the joining apparatus of the present disclosure will be explained. For convenience in explanation, the punch side will be referred to as the "upper side", the die side as the "lower side", a punch side metal sheet as an "upper side metal sheet", and a die side metal sheet as a "lower side metal sheet", but the joining apparatus is only required to be fastened in place. Standing, lying flat, or positioned in another direction is not important.

## Embodiment 1

FIGS. 1A and 1B are cross-sectional schematic views showing modes of mechanical joining using the mechanical joining apparatus of the present disclosure. FIG. 1A is a cross-sectional schematic view showing the state of starting to electrically heat a set of sheets at the same time as the start of an operation to drive in a rivet, while FIG. 1B is a cross-sectional schematic view showing the state after driving in the rivet.

As shown in FIG. 1A, in the mechanical joining apparatus 1, a punch 5 and a die 6 are arranged facing each other so as to be able to sandwich a set of sheets 4 comprised of an upper side metal sheet 2 and a lower side metal sheet 3 stacked together between them. At the outer circumference of the punch 5, a blank holder 7 is arranged.

The mechanical joining apparatus 1 is provided with a first power device (not shown) supplying current between the blank holder 7 and the die 6 so as to raise the temperature of the set of sheets 4 at the same time as the start of an operation to drive in a rivet 8 by the punch 5.

The "start of an operation to drive in a rivet 8" means the point of time when a rivet 8 to be driven in by the punch 5 contacts the punch side metal sheet of the set of sheets 4.

By electrically heating the set of sheets 4 at the same time as starting to drive in a rivet 8, it is possible to obtain a joint without fracture of the metal sheets, breakage of the rivet, and failure of rivet piercing. The set of sheets is heated after the start of the operation for driving in a rivet, so compared with the case of heating before driving it in, the heating region of the set of sheets can be easily limited to the joining

region and softening of the set of sheets at other than the joining region can be suppressed. For this reason, it is possible to prevent the set of sheets from changing in metal structure. In particular, when using as the metal sheet a 780 MPa or more high strength steel sheet, it is possible to join the steel sheet while keeping down a drop in strength.

The first power device is connected to the blank holder 7 and die 6 and is configured to electrically heat the set of sheets 4. The first power device may be provided with a first control device (not shown) controlling the amount of current (current value and application time) of the electric power supplied to the blank holder 7 and die 6 and can heat the set of sheets 4.

The first control device performs control to start to supply current to the blank holder 7 and die 6 to raise the temperature of the set of sheets 4 at the same time as starting the operation to drive in a rivet 8 and continues to supply current to the blank holder 7 and die 6 until the end of the operation to drive in the rivet 8 so as to electrically heat the set of sheets 4 to the desired temperature.

The electrical heating of the set of sheets 4 is started along with the start of the operation for driving in a rivet 8. The electrical heating of the set of sheets 4 may continue even after the end of the operation for driving in the rivet 8 and then stop, but preferably it stops substantially simultaneously with the end of the operation for driving in the rivet 8.

The "end of the operation for driving in a rivet 8" means the point of time when the punch substantially stops moving in the drive-in direction. It can be detected by detecting the position of the punch. The method of detecting the position of the punch is not particularly limited, but for example the position may be detected using a noncontact type laser displacement meter or a device detecting the position from the speed of a ball-screw pushing in the punch.

The driving speed of a rivet is preferably 1 mm/sec or more, more preferably 10 mm/sec. The rivet driving speed may be adjusted in accordance with the tensile strength etc. of the metal sheets of the set of sheets.

The time from the start of the operation for driving in a rivet 8 to the end of the operation may be adjusted depending on the material, thickness, number, etc. of the metal sheets used for the set of sheets. Preferably, it is 0.3 to 2.0 sec, more preferably 0.5 to 1.4 sec.

The heating temperature of the set of sheets 4 should be in a temperature range enabling the ductility of the set of sheets to be improved and suppressing fracture of the steel sheets or other metal sheets, breakage of the rivet, and failure of rivet piercing while enabling the rivet to be driven in. That is, the lower limit of the heating temperature of the set of sheets 4 should be made a temperature able to suppress fracture of the metal sheets, breakage of the rivet, and failure of rivet piercing. The upper limit of the heating temperature of the set of sheets 4 should be made a temperature of less than the melting point of the metal sheet with the lowest melting point among the set of sheets 4.

The lower limit of the heating temperature of the set of sheets 4 is preferably 400°C. or more, more preferably 500°C. or more, still more preferably 600°C. or more. The upper limit of the heating temperature of the set of sheets 4 is preferably 900°C. or less, more preferably 800°C. or less. The heating temperature of the set of sheets 4 is the temperature of the point of time of the end of the driving operation. It is measured at the location where the rivet is driven in at the surface of the upper side metal sheet in a region surrounded by the blank holder 7. The surface temperature of the upper side metal sheet can for example be measured using a thermocouple. The surface temperature of the upper side metal sheet may also be measured in advance before preparing the rivet. If measuring the surface temperature of the upper side metal sheet in advance, the measurement of temperature when using the punch to hold the rivet and drive it in may be eliminated.

The value of the current for electrically heating the set of sheets 4 may be controlled by the first control device so as to heat the set of sheets 4 to within the above temperature range within the time from the start of the operation for driving in the rivet to the end of the operation. The first control device can control the value of the current flowing through the set of sheets 4 to for example 8 to 14 kA or 10 to 12 kA. Further, the first control device can control the

current application time to substantially the same as the time from starting the operation for driving in the rivet 8 to the end of the operation.

The first control device can detect the time when the rivet 8 contacts the set of sheets 4 and control the first power device so as to start supplying current to the blank holder 7 and die 6. To detect the time when the rivet 8 contacts the set of sheets 4, for example, it is possible to use a voltmeter detecting a change in voltage between the punch 5 and die 6 when the rivet 8 contacts the set of sheets 4, a load cell built into the punch 5, etc.

The first power device is not particularly limited and may be a conventionally used power source, for example, a DC power device or AC power device.

The first control device is not particularly limited and may include a known thermostat. The first control device can use a thermostat including a thermometer for measuring the temperature of the set of sheets 4 and control the amount of electric power supplied through the blank holder 7 and die 6. It is also possible to find in advance the relationship between the current value and time giving the desired temperature corresponding to the combination of metal sheets of the set of sheets 4 and have the first control device control the current value and time to the same.

The punch 5 may be a rod shape. The cross-sectional shape in the direction vertical to the longitudinal direction of the punch 5 is not particularly limited and may be a circular shape, elliptical shape, rectangular shape, etc. The punch 5 may also have a cross-sectional shape different in the length direction.

The punch 5 is not particularly limited in its material so long as one having a strength enabling it to drive a rivet 8 in. It may be selected from materials having the desired mechanical strength. The punch 5 is preferably made of steel, copper, or copper alloy having a Vickers hardness Hv of 300 to 510. When using the punch as an electrode member as well, then punch 5 is preferably comprised of copper or copper alloy with a high electrical conductivity.

The die 6 is not particularly limited in material so long as being comprised of an electrode material having a mechanical strength and electrical conductivity enabling it to support a plurality of metal sheets and electrically heat the set of sheets 4. It may be selected from the desired materials. The die 6 is preferably copper or copper alloy.

At the outer circumference of the punch 5, the blank holder 7 is arranged. The blank holder 7 is a member which can contact the metal sheet at the punch 5 side of the set of sheets 4 at one end and press the set of sheets 4 against the die 6 and can move relatively to the punch 5 along its longitudinal axis. The blank holder 7 is shaped as a tubular member such as a tube into which the punch 4 is inserted.

The blank holder 7 is not particularly limited in material so long as it is made of an electrode material having mechanical strength and electrical conductivity enabling it to press a plurality of metal sheets against the die 6 and enabling it to electrically heat them. It may be selected from the desired materials. The blank holder 7 is preferably copper or copper alloy.

The copper alloy which can be used for the punch 5, die 6, blank holder 7, and cooling pipe 9 is preferably a chrome-copper alloy or alumina dispersed copper alloy. The composition of the chrome-copper alloy is preferably 0.4 to 1.6% Cr—Cu, more preferably 0.8 to 1.2% Cr—Cu, for example, 1.0% Cr—Cu, while the composition of the alumina dispersed copper alloy is preferably 0.2 to 1.0% Al<sub>2</sub>O<sub>3</sub>—Cu, more preferably 0.3 to 0.7% Al<sub>2</sub>O<sub>3</sub>—Cu, for example, 0.5% Al<sub>2</sub>O<sub>3</sub>—Cu.

A rivet **8** is placed at the front end of the punch **5**. This rivet **8** is driven into the set of sheets **4** by the punch **5**. A rivet for a general use part may be used or a full tubular rivet etc. may be used. The material of the rivet **8** is not particularly limited so long as the rivet can be driven into the set of sheets **4** to enable joining, but for example may be steel for mechanical structures, high hardness steel, etc.

Before the driving operation, the rivet **8** can be arranged above the set of sheets **4** in a state supported by the punch **5** or a state supported by a suitable support member.

The method of supporting the punch **5** by the rivet **8** or a suitable support member is not particularly limited, but for example it may be held mechanically or the punch **5** and support member may be made materials having magnetism and the rivet **8** may be magnetically attached to them.

The die **6** arranged facing the punch **5** may also have a dish-shaped or recessed-shaped upsetting surface **11** corresponding to the shape and size of the leg part of the rivet **8** which is driven in and may have a substantially frustoconical shaped projecting part **12** at its center. The top part of the projecting part **12** may be made slightly lower than the top surface of the die **6**. The base side of the projecting part **12** may have a smooth arc shaped surface connecting to the bottom surface of the upsetting surface **11**.

The set of sheets **4** in which a rivet is to be driven using the apparatus of the present disclosure may be comprised of two sheets of the upper side metal sheet **2** and lower side metal sheet **3** or may contain a plurality of three or more metal sheets. The metal sheets need only be ones which have flat parts at least in part and have parts enabling the flat parts to be stacked with each other. They do not have to be flat parts overall. Further, the set of sheets **4** is not limited to one comprised of separate metal sheets. A single metal sheet may be formed into a tubular shape or other predetermined shape and stacked.

The plurality of metal sheets may be the same types of metal sheets or may be different types of metal sheets. The metal sheets may be made metal sheets having a high strength. Steel sheet, aluminum sheet, magnesium, etc. may be used. The steel sheet is preferably high strength steel sheet, more preferably high strength steel sheet having a 780 MPa or more tensile strength. The plurality of metal sheets may include one or more steel sheets or may include one or more high strength steel sheets having a 780 MPa or more tensile strength. For example, the set of sheets **4** may be made a set of sheets where all of the metal sheets of the set of sheets **4** are made steel sheets, a set of sheets where the upper side metal sheet or lower side metal sheet is made high strength steel sheet and the other metal sheets are made steel sheets with a tensile strength of less than 780 MPa, a set of sheets where the upper side metal sheet is made aluminum and the lower side metal sheet is made high strength steel sheet, or a set of sheets where the metal sheets of all of the set of sheets **4** are made aluminum sheets. If using the apparatus of the present disclosure, it is possible to join well a set of sheets including at least one high strength steel sheet with a 780 MPa or more tensile strength.

The thickness of the metal sheets is not particularly limited. For example, it may be made 0.5 to 3.0 mm. Further, the thickness of the set of sheets is also not particularly limited. For example, it may be made 1.0 to 6.0 mm. Further, the presence of plating, the chemical composition, etc. are also not particularly limited.

FIGS. 1A and 1B illustrate the flow of current from the blank holder **7** toward the die **6** by the dot-chain lines, but it is sufficient that the set of sheets **4** be able to be electrically

heated. It is also possible to make the current flow from the die **6** toward the blank holder **7**. The same is true in FIGS. 2A and 2B and 3A and 3B.

## Embodiment 2

As a preferable embodiment, Embodiment 2 will be explained. The joining apparatus of the present disclosure is preferably further provided with a cooling device (not shown).

The cooling device is connected to the punch **5** and is configured to cool a rivet **8** through the punch **5** in the period from the start of the operation for driving in a rivet **8** to the end of the operation. The set of sheets **4** is electrically heated while using the cooling device connected to the punch **5** to cool the rivet **8** while driving in the rivet **8** by the punch **5** to thereby join the set of sheets **4**.

By electrically heating the set of sheets **4** between the blank holder **7** and the die **6** while cooling the rivet **8** through the punch **5** when driving in the rivet **8**, it is possible to suppress softening of the rivet **8** due to the heat of the set of sheets **4** and possible to more stably perform the riveting. By cooling the rivet **8**, even when in particular the temperature of the set of sheets **4** when driving in the rivet **8** is high, it is possible to keep the rivet **8** from softening and prevent failure of piercing of the rivet **8** and thereby enable more stable joining.

The rivet **8** may be cooled in the period from the start of the operation to drive in a rivet **8** to the end of the operation. That is, the rivet **8** may be cooled starting from before the operation for driving it in or may be started simultaneously with the start of the operation for driving it in, but preferably the rivet **8** starts to be cooled from before the operation for driving it in. The rivet **8** may finish being cooled simultaneously with the end of the operation for driving it in or may continue to be cooled even after the end of the operation for driving it in, but preferably it is ended substantially simultaneously with the end of the operation for driving it in.

The cooling device is not particularly limited so long as one able to cool the rivet **8** through the punch **5**, but the punch **5** may also have a cooling pipe **9** inside it. FIG. 1A shows a cooling pipe **9** arranged inside the punch **5** and connected to the cooling device.

The cooling pipe **9** is a pipe able to supply coolant in for example the direction shown by the arrows. A cooling device connected to the cooling pipe **9** at the other end side at the opposite side to the end of the punch **5** which the rivet **8** contacts can be provided. The cooling pipe **9** is not particularly limited in material so long as it can carry the coolant inside and cool the rivet through the punch **5**, but for example it may be made of copper or a copper alloy. In this case, the punch **5** is preferably made copper or a copper alloy with a high heat conductivity.

The coolant is not particularly limited. A known liquid coolant or gaseous coolant may be used, but if considering economy and ease of handling etc., water is preferable.

It is also possible not to provide a cooling pipe **9** inside the punch **5** but to arrange the cooling device so as to contact the other end part at the opposite side to the end part of the punch **5** which the rivet **8** contacts and cool the punch **5** so as to cool the rivet **8** by heat conduction of the punch **5**. In this case as well, the punch **5** is preferably made of copper or copper alloy with a high heat conductivity.

The rivet **8** should be cooled in the period from the start of the operation for driving in a rivet **8** to the end of the operation. That is, the rivet **8** may start to be cooled from before the operation for driving in the rivet **8** or may start to

## 11

be cooled simultaneously with the start of the operation, but preferably the rivet **8** starts to be cooled from before being driven in. The rivet **8** may finish being cooled simultaneously with the end of the operation for driving in the rivet or may continue to be cooled even after the end of the operation, but preferably it ends substantially simultaneously with the end of the operation for driving in the rivet.

The cooling device is provided with a control device which can control the cooling temperature and the timing of the start and end of the cooling. The control device controls the cooling device so that the temperature of the rivet **8** becomes preferably 3 to 50° C., more preferably 5 to 30° C., preferably at the time of the end of the operation for driving in the rivet, more preferably from the start of the operation for driving in the rivet to the end of the operation. The temperature of the rivet **8** may be found, for example, before actual joining, by conducting a preliminary test for measurement of the temperature of the rivet in advance and using a thermocouple to measure the temperature of the rivet. The control device provided at the cooling device is not particularly limited and may include a known thermostat.

## Embodiment 3

Referring to FIGS. 2A and 2B, the preferred embodiment of Embodiment 3 will be explained. FIGS. 2A and 2B are cross-sectional schematic views showing the modes of mechanical joining using the mechanical joining apparatus of the present disclosure. FIG. 2A is a cross-sectional schematic view showing the state of electrically heating the set of sheets at the same time as the start of the operation for driving in a rivet, while FIG. 2B is a cross-sectional schematic view showing the state of electrically heating the rivet after driving in the rivet.

The mechanical joining apparatus **1** is provided with a second power device (not shown) for supplying current through the punch **5** and die **6** so that the rivet **8** driven in by the punch **5** is heat treated. The mechanical joining apparatus of FIG. 2 has a configuration similar to the mechanical joining apparatus of FIG. 1 except that the punch **5** and die **6** are comprised of electrode materials and the rivet **8** can be electrically heated.

The second power device is connected to the punch **5** and die **6** and is configured to supply current to the rivet **8** through the punch **5** and die **6** so as to heat treat it after the punch **5** drives in the rivet **8**. The second power device may be provided with a second control device (not shown) controlling the amount of electric power supplied through the punch **5** and die **6** (current value and application time) so as to heat the rivet **8** to the desired temperature.

The cooling device connected to the second power device and punch **5** may be used for heat treatment for heating the rivet **8** to the austenite region after the end of the operation for driving in the rivet **8**, then cooling it. Due to this, the rivet **8** may be given a martensite structure and the strength of the rivet **8** may be improved. The cooling device used in the Embodiment 3 may be the same as or different from the cooling device used in the Embodiment 2.

By heat treating the rivet **8** after it finishes being driven in so as to raise the strength, it is possible to reduce more the breakage of a rivet and area around it of the joint obtained using a rivet.

In particular, even when joining a set of sheets including high strength steel sheet and a rivet for general use parts not high in strength, it is possible to suppress stress from

## 12

concentrating at the low strength rivet and more stably prevent breakage of the joint obtained by using a rivet.

To increase the strength of a rivet, in the past, the art of adjusting the chemical composition and heat treating the rivet by hardening etc. has been known (PLT 3). However, in this art, there were the problems that the rivet is limited in chemical composition, a heat treatment furnace becomes necessary for the heat treatment, the costs rise, further, a heat treatment process in the heat treatment furnace becomes necessary, and an increase in the production time of the rivets is invited.

As opposed to this, it is possible to use the punch and die for driving in the rivet as electrode members and supply a current to the rivet driven into the set of sheets to electrically heat and heat treat the rivet, that is, heat the rivet made of a steel material for general part use to the temperature where it becomes the austenite region, then rapidly cool it to obtain a martensite structure and thereby make the rivet high in strength. For this reason, it is possible to obtain a high strength rivet without using a heat treatment furnace etc.

The heating temperature in the heat treatment of the rivet **8** is not particularly limited so long as one enabling the rivet **8** to be heated to the austenite region, but preferably the A3 point to a temperature of less than the melting point of the rivet is heated to. The current value and time in heating the rivet **8** to its highest temperature may be for example a current value of 8 to 10 kA and a time of 0.1 to 1.0 sec.

The operation for electrically heating a rivet **8** may be started simultaneously with the end of the operation for driving in the rivet **8** or after the elapse of a predetermined time from the end of the operation for driving in the rivet **8**. The second control device may control the second power device so as to electrically heat the rivet **8** simultaneously with the end of the operation for driving in the rivet **8** or after the elapse of a predetermined time from the end of the operation for driving in the rivet **8**.

The cooling conditions after heating a rivet **8** to the austenite region are not particularly limited so long as a martensite structure is obtained, but the control device provided at the cooling device may control the cooling device so that after the rivet **8** is heated to the austenite region, the rivet **8** is preferably cooled by a 10° C./sec or more cooling speed down to the martensite transformation end temperature or less of the material forming the rivet, in general, down to about 200° C. or less.

When cooling the rivet **8** through the punch **5** at the time of the operation for driving in a rivet **8**, it is possible to continue to cool the rivet **8** through the punch **5** while heat treating the rivet **8** after the operation for driving in the rivet **8** so long as the electrical heating enables the rivet **8** to be heated to a predetermined temperature, but preferably the punch **5** stops being cooled or the amount of cooling is reduced and, after heat treating the rivet **8**, the cooling is resumed or the amount of cooling is increased to thereby cool the rivet **8**.

The punch **5** is not particularly limited in material so long as it is made from an electrode material having mechanical strength and electrical conductivity enabling a rivet **8** to be driven in and enabling electrical heating. It may be selected from the desired materials. The punch **5** preferably is comprised of copper or a copper alloy having a Vickers hardness Hv of 300 to 510 and having a high electrical conductivity.

The die **6** is not particularly limited in material so long as it is made from an electrode material having mechanical strength and electrical conductivity able to support a plurality of metal sheets and able to electrically heat the set of

## 13

sheets 4 and rivet 8. It may be selected from the desired materials. The die 6 is preferably copper or a copper alloy. The die 6 may be configured by the same material as that used in the Embodiment 1.

The second power device is not particularly limited and may be a power source used in the past such as a DC power device or AC power device. The second power device may also be configured in the same way as the first power device.

The second control device is not particularly limited and may include a known thermostat. The second control device may use a thermostat including a thermometer for measuring the temperature of a rivet 8 so as to control the amount of current supplied through the punch 5 and die 6. The relationship between the current value where the rivet 8 becomes a predetermined temperature and the time may be found in advance and the second control device may control the second power device so as to obtain that current value and time.

The control device provided at the cooling device may use a thermostat to control the cooling speed and cooling temperature after heat treatment of the rivet 8.

The first power device and the second power device may be made separate power devices or an integrated power device or the first power device may also have the function of the second power device.

When the first power device and second power device are formed from an integrated power device or when the first power device also has the function of the second power device, that power device is connected to both of the blank holder 7 and die 6 and the punch 5 and die 6.

## Embodiment 4

Referring to FIGS. 3A and 3B, the preferred embodiment of the Embodiment 4 will be explained. FIGS. 3A and 3B are cross-sectional schematic views showing the modes of mechanical joining using a mechanical joining apparatus provided with tool steel as part of the die. FIG. 3A is a cross-sectional schematic view showing the state of electrically heating a set of sheets before driving in a rivet when using tool steel for part of the die, while FIG. 3B is a cross-sectional schematic view showing the state of electrically heating a rivet after driving in a rivet when using tool steel for part of the die. The mechanical joining apparatus of FIGS. 3A and 3B has a configuration similar to the mechanical joining apparatus of FIGS. 2A and 2B except for the fact that the die 6 is comprised of a die made of tool steel 6a and a die made of copper or copper alloy 6b.

To suppress deformation of the die, in the die, it is effective to increase the strength of the part facing the rivet across the set of sheets 4 (part below part where rivet 8 is to be driven in). For this reason, as shown in FIGS. 3A and 3B, by making the part in the die 6 restraining the lower side metal sheet 3, which can deform due to the rivet 8 being driven in, a die 6a made of tool steel, it is possible to increase the strength of the die 6 and possible to suppress deformation of the die 6.

When driving a rivet into the set of sheets, if supplying current between the blank holder and the die or supplying current between the punch and die so as to heat treat the driven in rivet, the die is heated. At this time, if the die is made completely of tool steel, the die will easily soften. For this reason, preferably, the outer circumference part of the die 6a made of tool steel is comprised of copper or copper alloy from the viewpoint of facilitating the flow of current.

By placing the die 6b made of copper or copper alloy low in electrical resistance so as to surround the outer circum-

## 14

ference part of the die 6a made of tool steel, when supplying current between the blank holder 7 and the die 6 or supplying current between the punch 5 and the die 6, the current flows with priority to the outer circumference part with the low electrical resistance, so the die 6a made of tool steel becomes hard to heat and softening can be prevented.

When configuring part of the die 6 by tool steel, in the die 6, it is sufficient that at least the part facing the rivet 8 across the set of sheets 4 be comprised of tool steel, but just a portion of the part facing the blank holder 7 across the set of sheets 4 may also be comprised of tool steel. However, in the die 6, as the ratio of the part comprised of copper or copper alloy becomes smaller, current flows through the tool steel and the tool steel easily softens, so it is possible to adjust the ratio of the part comprised of the tool steel and the part comprised of copper or copper alloy in accordance with the amount of current flowing between the blank holder 7 and die 6 or between the punch 5 and die 6.

The present disclosure further, covers a mechanical joining method using a punch to drive a rivet into a plurality of metal sheets, the mechanical joining method comprising

preparing a plurality of metal sheets,

placing the plurality of metal sheets stacked between a punch and die arranged facing each other,

pushing one end of a blank holder comprised of a tubular member inside of which the punch can be inserted against a punch side metal sheet of the plurality of metal sheets,

using the punch to drive a rivet into the plurality of metal sheets held by the blank holder, and

starting to electrically heat the plurality of metal sheets through the blank holder and the die so as to raise the temperature of the plurality of metal sheets at the same time as the start of the driving in of the rivet and continuing to electrically heat the plurality of metal sheets until the end of the driving in of the rivet (below, also referred to as "the joining method").

The joining method of the present disclosure will be explained while referring to FIGS. 1A and 1B.

A set of sheets 4 of a plurality of metal sheets is prepared. The set of sheets 4 may include at least one high strength steel sheet with a tensile strength of 780 MPa or more and may also include only metal sheets with tensile strengths of less than 780 MPa.

The set of sheets 4 is placed on the die 6, one end of the blank holder 7 comprised of a tubular member is pushed against the punch 5 side metal sheet of the set of sheets 4, and the punch 5 is used to drive in a rivet 8 into the set of sheets 4 pushed down by the blank holder 7.

To raise the temperature of the set of sheets 4, at the same time as the start of the operation for driving in a rivet 8, current starts to be supplied through the set of sheets 4 through the blank holder 7 and die 6. It continues to be supplied through the set of sheets 4 until the end of the operation for driving in the rivet 8.

Preferably, in the period from the start of the operation for driving in a rivet 8 to the end of the operation, the rivet 8 is cooled through the punch 5.

Preferably, after driving in the rivet, the rivet is electrically heated through the punch and die to heat treat it.

Preferably, in the die, at least the part facing the rivet across the plurality of metal sheets is made of tool steel while the part at the outer circumference of the tool steel is made of copper or copper alloy.

Preferably, the blank holder has a through hole into which the punch can be inserted, and the punch is made to slide with the through hole while making it move relative to the blank holder.

## 15

Preferably, the other end of the blank holder is provided with an elastic member, and the elastic member applies a pressing pressure through the blank holder to the plurality of metal sheets.

The punch 5 can be made to move by a movement device (not shown) so that the blank holder 7 moves together with the punch 5 through the compression coil spring 14 and contacts the set of sheets 4. To ensure the steel sheets of the set of sheets 4 closely contact, a pressing force of an extent whereby the rivet 8 stops at a position not contacting the set of sheets 4 may be used to make the blank holder 7 move with respect to the die 6.

For the configuration of the joining method of the present disclosure, it is possible to apply the configuration explained with reference to the mechanical joining apparatus.

## EXAMPLES

## Example 1

Using the mechanical joining apparatus 1 shown in FIGS. 1A and 1B, as a joining test in the case of a large deformation resistance of the metal sheets, a joining test of a set of sheets including one or more high strength steel sheets with a tensile strength of 780 MPa or more was performed.

A set of sheets 4 including, as a high strength steel sheet with a tensile strength of 780 MPa or more, a thickness 1.2 mm steel sheet with a 980 MPa tensile strength as an upper side metal sheet and, as a steel sheet with a tensile strength of less than 780 MPa, a thickness 1.6 mm steel sheet with a 440 MPa tensile strength as a lower side metal sheet was prepared.

As shown in FIG. 1A, the set of sheets 4 was placed on the copper die 6 then the copper blank holder 7 was used to push down the set of sheets 4 to make the sheets closely contact each other. As the rivet 8, a full tubular rivet made of high hardness steel and having a diameter of 6 mm was prepared and held at the punch 5.

Using a riveting speed of 10 mm/sec, a 1.0% Cr—Cu punch 5 was used to start to drive the rivet 8 into the set of sheets 4. Simultaneously with this, 10 kA current was supplied for 1.0 second between the blank holder 7 and die 6 using a first power device provided with a first control device so as to heat the set of sheets 4 and the rivet 8 was driven in. The temperature of the set of sheets 4 after the rivet finished being driven in was 750° C. A joined part such as shown in FIG. 1B was obtained, the stacked steel sheets were completely closely in contact, and the set of sheets could be joined without fracture of the metal sheets, breakage of the rivets, or failure of rivet piercing.

## Example 2

Except for preparing, as the set of sheets comprised of metal sheets with a tensile strength of less than 780 MPa, an upper side metal sheet and lower side metal sheet comprised of metal sheets having 590 MPa and 440 MPa tensile strengths, increasing the rivet driving speed to 20 mm/sec, and supplying a 20 kA current for 0.5 second, a joining test was conducted under conditions similar to Example 1. The set of sheets could be joined without fracture of the metal sheets, breakage of the rivet, or failure of rivet piercing.

## Example 3

Except for using a punch 5 provided inside it with a cooling pipe 9 connected to a cooling device provided with

## 16

a thermostat and shown in FIG. 1 to cool the rivet 8 through the punch 5 to 30° C. while driving in the rivet 8 by the punch 5 and for heating the set of sheets 4 to 780° C., a joining test was conducted under conditions similar to Example 1. The set of sheets could be joined without fracture of the metal sheets, breakage of the rivet, or failure of rivet piercing.

## Example 4

Except for using the mechanical joining apparatus 1 shown in FIG. 2 to heat treat and cool the rivet 8 after driving in the rivet 8, a joining test was conducted under conditions similar to Example 3.

After the end of the driving operation, the rivet 8 stopped being cooled and the set of sheets 4 stopped being heated. 8 kA current was supplied through the punch 5 and die 6 using a second power device provided with a thermostat for 0.5 second to heat the rivet 8 to the austenite region of 900° C., then this was rapidly cooled by a 30° C./sec cooling rate down to 180° C. by a cooling device provided with a thermostat.

When the heat treated rivet was examined, it was confirmed that it had a martensite structure. Further, when conducting a joint strength test on the joint, it was learned that breakage of the rivet and area around it was decreased more compared with the case of not heat treating the rivet.

## Example 5

Except for using the mechanical joining apparatus 1 shown in FIG. 3, making the part facing the rivet 8 across the set of sheets 4 a die made of tool steel 6a, and placing a copper die 6b at the outer circumference part of the die 6a, a joining test was conducted under conditions similar to Example 1. It was possible to suppress deformation of the die 6 and the set of sheets could be joined without fracture of the metal sheets, breakage of the rivet, or failure of rivet piercing.

## REFERENCE SIGNS LIST

1. mechanical joining apparatus
2. upper side metal sheet
3. lower side metal sheet
4. set of sheets
5. punch
- 5a. contact part of punch
- 5b. sliding part of punch
6. die
- 6a. die made of tool steel
- 6b. die made of copper or copper alloy
7. blank holder
8. rivet
9. cooling pipe
10. through hole
11. upsetting surface
12. projecting part
13. movable plate
14. holder
15. compression coil spring
16. holding plate
17. plastic member
18. guide bolt

The invention claimed is:

1. A mechanical joining method using a punch to drive a rivet into a plurality of metal sheets, the mechanical joining method comprising

preparing a plurality of metal sheets,

placing the plurality of metal sheets stacked between a punch and a die arranged facing each other,

pushing one end of a blank holder comprised of a tubular member inside of which the punch can be inserted against a punch side metal sheet of the plurality of metal sheets,

using the punch to drive a rivet into the plurality of metal sheets held by the blank holder,

starting to electrically heat the plurality of metal sheets through the blank holder and the die so as to raise the temperature of the plurality of metal sheets at the same time as the start of the driving in of the rivet through the metal sheets and continuing to electrically heat the plurality of metal sheets until the end of the driving in of the rivet, and

cooling the rivet through the punch in a period from the start of the driving in of the rivet until the end of the driving in of the rivet.

2. The mechanical joining method according to claim 1, further comprising, after driving in the rivet, electrically heating the rivet through the punch and the die to heat treat the rivet, then cooling the rivet.

3. The mechanical joining method according to claim 2, wherein in the die, at least a part facing the rivet across the plurality of metal sheets is made of tool steel and a part at the outer circumferences of the tool steel is made of copper or copper alloy.

4. The mechanical joining method according to claim 1, wherein in the die, at least a part facing the rivet across the plurality of metal sheets is made of tool steel and a part at the outer circumferences of the tool steel is made of copper or copper alloy.

5. A mechanical joining method using a punch to drive a rivet into a plurality of metal sheets, the mechanical joining method comprising

preparing a plurality of metal sheets,

placing the plurality of metal sheets stacked between a punch and a die arranged facing each other,

pushing one end of a blank holder comprised of a tubular member inside of which the punch can be inserted against a punch side metal sheet of the plurality of metal sheets,

5

10

15

20

25

30

35

40

using the punch to drive a rivet into the plurality of metal sheets held by the blank holder,

starting to electrically heat the plurality of metal sheets through the blank holder and the die so as to raise the temperature of the plurality of metal sheets at the same time as the start of the driving in of the rivet through the metal sheets and continuing to electrically heat the plurality of metal sheets until the end of the driving in of the rivet, and

after driving in the rivet, electrically heating the rivet to the austenite region through the punch and the die, then cooling the rivet down to 200° C. or less by a 10° C./sec or more cooling speed in order to obtain martensite structure in the rivet.

6. The mechanical joining method according to claim 5, wherein in the die, at least a part facing the rivet across the plurality of metal sheets is made of tool steel and a part at the outer circumferences of the tool steel is made of copper or copper alloy.

7. A mechanical joining method using a punch to drive a rivet into a plurality of metal sheets, the mechanical joining method comprising

preparing a plurality of metal sheets,

placing the plurality of metal sheets stacked between a punch and a die arranged facing each other,

pushing one end of a blank holder comprised of a tubular member inside of which the punch can be inserted against a punch side metal sheet of the plurality of metal sheets,

using the punch to drive a rivet into the plurality of metal sheets held by the blank holder, and

starting to electrically heat the plurality of metal sheets through the blank holder and the die so as to raise the temperature of the plurality of metal sheets at the same time as the start of the driving in of the rivet through the metal sheets and continuing to electrically heat the plurality of metal sheets until the end of the driving in of the rivet,

wherein in the die, at least a part facing the rivet across the plurality of metal sheets is made of tool steel and a part at the outer circumferences of the tool steel is made of copper or copper alloy.

\* \* \* \* \*